

## UNITED STATES PATENT OFFICE

BORIS N. LOUGOVY, OF MONTCLAIR, NEW JERSEY, ASSIGNOR TO CHADELOID CHEMICAL COMPANY, OF NEW YORK, N. Y., A CORPORATION OF WEST VIRGINIA

## PAINT AND VARNISH REMOVER CONTAINING FURFURAL

No Drawing.

Application filed June 18, 1928. Serial No. 286,496.

This invention relates to paint and varnish removers containing furfural and especially to this solvent incorporated with other solvents with or without a thickening agent and further relates to an incorporation of this solvent with certain other solvents, illustratively an alcohol and a chlorinated hydrocarbon in order to produce a highly efficient paint and varnish remover having certain characteristics which differentiate from other paint and varnish removers in several useful respects.

When applied by itself furfural drains off of vertical surfaces and the action is aggravated by the fact that this solvent does not wet the surface readily but tends to gather in drops. The addition of an auxiliary or co-operative solvent such as alcohol, benzol, toluol and various chlorinated solvents, such as carbon tertachloride, acetylene tetrachloride, trichlorethylene and particularly monochlorbenzol may be used to overcome the difficulty of lack of surface wetting, to some extent.

To give body or consistency to the composition a thickener may be incorporated including wax, soap and various other thickeners such as esters of cellulose in some cases. Wax is especially serviceable to retard the evaporation of volatile solvents and for this purpose paraffin or ceresin wax (mineral wax) is best. Furfural is slow to evaporate but may be incorporated with more volatile solvents which require repression of evaporation to confine them to the surface to be softened. The proportion of the wax in fact depends on the nature of the solvents used but, generally, it is better to employ as little wax as possible, particularly if the remover is used to clean off a surface which is afterwards to be coated with nitro-cellulose lacquer.

Not all volatile solvents are adapted to be used with furfural, gasoline and petroleum naphtha of themselves not being miscible and furthermore not possessing any satisfactory paint and varnish removing qualities. To secure good results solvents which are miscible should be chosen or if an immiscible solvent is to be included the addition of blend-

ing solvents sometimes will bring about miscibility. In general the requirements of a paint and varnish remover of a commercial character necessitate the employment of solvents of strong cutting qualities and the addition of substantial proportions of indifferent solvents tends to produce a low grade remover of unsatisfactory qualities incapable of reaching commercial standards.

The speed of a commercial remover, that is, the shortness of time required to soften the coat of paint or varnish, is very essential from a practical standpoint because a fast powerful remover not only will save time in the removal of the paint from a given surface but also will save some expense in the consumption of materials.

The activity of a paint and varnish remover is usually tested in the trade by a means which is not absolutely reliable but nevertheless is regarded sufficiently convincing to the user. The method involves the application of some of the removing composition to a surface coated with a paint or varnish and to note the time taken for the surface to wrinkle. This wrinkling effect is regarded as an indication of the solvent action or "cutting power" of the removing composition.

The method adopted when working on the present problem to determine the cutting power was as follows: A piece of old painted wood was selected, taking care that the portion used had a good even, thick coat of paint. This was cut into strips. Various solvents were placed in a series of test tubes and a strip of the painted wood was put into each test tube. The time which elapsed before the first appearance of any wrinkling was accurately noted for each solvent by means of a stop watch. The comparative "removing action" or "cutting power" was thus roughly represented by the number of elapsed seconds.

Solvent mixtures vary greatly in cutting power. In removers involving the use of a penetrating hydrocarbon such as benzol and a loosening solvent of an alcoholic or ketonic nature a very great variation is observable in the cutting action depending upon the solvents employed.

50

60

65

70

75

76

80

85

90

95

100

In regard to removing action furfural by itself has relatively only mild dissolving power and as already stated possesses the disadvantage of draining off of vertical surfaces. 5 In addition, I have observed that furfural in most mixtures with other solvents also possesses the rather undesirable property of "slow initial action", that is, when applied to a painted surface the mixture acts very 10 slow at the beginning in comparison with non-furfural mixtures with other loosening solvents. On the other hand when furfural is used, and the cutting action starts, it progresses rapidly. In order to produce a 15 remover with a high speed of initial attack I find it necessary to correct this peculiar disadvantage of furfural.

In the course of my investigations on paint and varnish removers, I discovered that a 20 combination of furfural, monochlorbenzol and anhydrous methyl alcohol is surprisingly advantageous. A combination of those three solvents produces a very fast-acting removing composition. I also observed that as soon 25 as either one of the above three ingredients was omitted from the mixture and replaced with some other solvent, even of a similar character, the activity or efficiency of the remover immediately dropped in greater or 30 lesser degree.

In an effort to secure the quickest possible action for a paint and varnish remover I proceeded first with the investigations of the cutting power of various single solvents of 35 different natures, turning them to a mixture of two solvents, three solvents, and so forth. In this investigation many interesting facts have been observed which are illustrated in the tabulation below in connection with the 40 furfural-containing compositions, the tests being conducted on painted strips as described above:

Table 1

|                                              | Cutting power-seconds |
|----------------------------------------------|-----------------------|
| Furfural                                     | 300                   |
| Monochlorbenzol                              | 400                   |
| Anhydrous methyl alcohol                     | 240                   |
| Furfural and monochlorbenzol                 | 50                    |
| 50 Furfural and benzol                       | 90                    |
| Furfural and anhydrous methyl alcohol        | 35                    |
| Furfural and acetone                         | 40                    |
| Furfural-ethyl alcohol (95%)                 | 70                    |
| Furfural-ethyl alcohol (anhydrous)           | 55                    |
| 55 Furfural-trichlorethylene                 | 50                    |
| Furfural-benzol-methanol (anhydrous)         | 45                    |
| Furfural-benzol-methyl acetate               | 35                    |
| Furfural-benzol-acetone                      | 55                    |
| 60 Furfural-monochlorbenzol-methanol (anhy.) | 5                     |
| Furfural-monochlorbenzol-methyl acetate      | 15                    |

In the above mixtures of various solvents equal volumes of each component solvent are used in all cases.

Throughout this present description, the terms "methanol" and "methyl alcohol" are used in a synonymous manner, and the tests herein all refer to the anhydrous material, in order to be comparative. Anhydrous methanol is superior to the product containing 5 to 10% or so of water.

The term "methyl solvent" as hereinafter employed is intended to embrace methyl alcohol and methyl acetate, which as shown in the above Table 1, are both highly effective in removers of the present invention.

It is understood that all formulas given below should be regarded only as examples and that I do not wish to restrict myself to the exact proportions given in these formulas. All these examples will include in the formulas paraffin wax as an agent to retard evaporation of the solvents for comparison (but without restricting the invention) and in some cases will also include nitrocellulose (scrap celluloid) as an agent to increase the consistency of the paint and varnish remover. It should be noted in this connection that the addition of various solids which are capable of dissolving in one of the solvents used in paint and varnish remover generally will result in cutting down of the speed of a given solvent or of a mixture of this solvent with other solvents, and therefore the cutting speed or rate of attack of wax-containing compositions will be slower than the cutting speed of a corresponding mixture without a wax.

The figures in Table 2, which refer to composition of removers, represent the amount of each ingredient by volume including wax (which is reported as measured in the molten state). Table 2 sets forth the cutting speed of each composition in the number of seconds necessary to produce wrinkling of a given painted surface. For this purpose a part of an old automobile (finished with an oil paint) was utilized. Each remover was placed on the surface in approximately the same quantity and the time was noted by means of a stop watch when the blistering or wrinkling of the surface was plainly observable.

In order that a paint and varnish remover have a practical value in addition to its efficiency or power to penetrate the paint it should also possess the property of remaining wet for a long period. The retardation of evaporation, as already mentioned, is usually accomplished by introducing into the removing composition a certain amount of wax or other film-forming substance. However, the relative amount of such agent is limited due to the fact, which has already been mentioned, that any solid substances introduced into the remover generally will decrease its activity. The rate of evaporation of paint and varnish removers in part depends not only upon the relative amount of material used to arrest evaporation, but also

in a large degree upon the boiling point and vapor pressure of solvents included in the remover. The boiling point of each individual solvent is of importance as well as the ratio between the boiling point and/or the vapor pressure of wax solvent to the boiling point and/or the vapor pressure of wax precipitant. As a general rule the wax precipitant should be the less volatile body.

From the standpoint of rate of evaporation a remover welcome for practical use will be one which loses not over about 5% of its weight in, say, twenty-four hours. Remover applied in the afternoon then will be found on the following morning to have penetrated even very obstinate coatings and to have softened or jellified them for ready removal with wire brush or putty knife.

Data regarding loss in weight of the furfural-containing removers therefore are included in Table 2.

Table 2.—Composition of typical removers (parts all by volume)

| Solvents                              | 1   | 2   | 3   | 4   | 5   | 6    | 7   | 8   | 9          | 10 | 11   | 12  | 13  | 14  |
|---------------------------------------|-----|-----|-----|-----|-----|------|-----|-----|------------|----|------|-----|-----|-----|
| Dichlorbenzol.                        |     |     |     |     |     |      |     |     |            |    |      |     |     |     |
| Monochlorbenzol.                      | 40  |     | 40  | 40  | 40  | 40   | 40  | 40  | 40         | 40 | 40   | 40  | 40  | 50  |
| Benzol.                               |     | 40  | 40  |     |     |      |     |     |            |    |      |     |     |     |
| Furfural.                             | 20  | 20  | 20  | 20  | 20  | 20   |     |     |            | 30 | 20   | 20  | 25  | 50  |
| Methanol.                             | 20  | 20  | 20  |     |     | 20   | 20  | 25  | 25         | 30 | 20   | 20  | 25  | 50  |
| Acetone.                              |     |     | 20  | 20  |     | 20   | 20  | 15  |            |    |      |     |     |     |
| Lugosol.                              |     |     |     |     |     |      |     |     | 15         |    | 20   |     |     |     |
| Methyl acetate.                       | 20  | 20  | 20  | 20  | 20  | 20   | 15  | 15  |            |    | 20   |     |     |     |
| Wax.                                  | 2   | 2   | 2   | 2   | 2   | 2    | 3   | 3   | 2          | 2  | 2    | 2   | 2   | 4   |
| Trichlorethylene.                     |     |     |     |     |     |      |     |     |            | 40 | 60   |     |     |     |
| Comparative cutting speed in seconds. | 45  | 115 | 130 | 240 | 150 | 55   | 130 | 120 | 100        | 70 | 60   | 100 | 120 | 300 |
| Loss in weight in 24 hours (%)        | 1.4 | 3.2 | 4.3 | 4.4 | 5.5 | 10.0 | 3.2 | 6.0 | Not tested | 20 | 12.5 | 1   |     |     |

Examination of the above table shows that in order to secure the fastest acting compositions it is necessary to use all three solvents, viz: monochlorbenzol, furfural and anhydrous methanol simultaneously. The addition of some other solvent of either ketonic or esteric nature will only increase the absolute value of the removing power within a comparatively narrow limit. Example 1, representing a combination giving the fastest remover, includes methyl acetate in addition to the above three basic solvents. Replacement of methyl acetate with acetone, as in Example 6, causes the absolute speed of the remover to drop slightly but the composition will still remain faster than any other composition from which one of the three basic solvents has been omitted, as for instance compositions in Examples 4 and 7. The other mixtures are grouped as follows: Examples 2 and 3 represent mixtures in which monochlorbenzol is omitted. Examples 4 and 5 represent mixtures in which anhydrous methanol is omitted. Examples 7, 8 and 9 represent mixtures in which furfural is omitted and Examples 1, 6, 10 and 11 represent mix-

tures containing all three basic solvents together.

These figures are by no means absolute but serve to indicate in a general way the advantages of using with furfural a solvent of the monochlorbenzol type in conjunction with a methanolic solvent yielding a remover possessing high initial surface wrinkling power capable of rapidly opening the surface to the ingress of solvent. Such a remover offers a considerable saving in time in the cleaning off of painted surfaces, especially those where by the effect of long exposure to the air, the outer layer of the coating is oxidized to a state of high resistivity to solvent action.

While I have found anhydrous methyl alcohol to be the most advantageous co-operating solvent with furfural especially as a potent surface-opening agent, I do not limit myself to this surface-opening activator but may include other highly volatile solvents containing the methyl group such as methyl acetate and the like.

What I claim is:

1. A high speed paint and varnish remover possessing high initial surface wrinkling power capable of rapidly opening the surface to ingress of solvent, said remover containing furfural, methanol, chlorinated hydrocarbons miscible therewith, and a wax.

2. A high speed paint and varnish remover possessing high initial surface wrinkling power capable of rapidly opening the surface to ingress of solvent, said remover comprising furfural, monochlorbenzol, anhydrous methanol and a wax.

3. A high speed paint and varnish remover possessing high initial surface wrinkling power capable of rapidly opening the surface to ingress of solvent, said remover comprising fulfural, chlorbenzol, anhydrous methanol and a thickening agent.

4. A high speed paint and varnish remover possessing high initial surface wrinkling power capable of rapidly opening the surface to ingress of solvent said remover containing furfural, chlorbenzol, methyl alcohol, and a wax.

5. A high speed paint and varnish remover possessing high initial surface wrinkling power capable of rapidly opening the surface to ingress of solvent, said remover containing furfural, a wax solvent selected from the group consisting of benzol, toluol and chlorbenzol, methyl alcohol, and a wax.

6. A finish remover comprising furfural, a methyl solvent selected from the herein described group consisting of methyl alcohol and methyl acetate, an aromatic chlorinated single ring hydrocarbon wax solvent, and a wax.

7. A finish remover comprising furfural and anhydrous methyl alcohol.

8. A finish remover comprising furfural and a highly volatile methyl solvent selected

from the herein described group consisting of methyl alcohol and methyl acetate, a wax solvent and wax.

9. A high speed paint and varnish remover possessing high initial surface wrinkling power capable of rapidly opening the surface to ingress of solvent, said remover containing furfural, a benzolic solvent selected from the group consisting of benzol and chlorbenzol, a methyl solvent selected from the group consisting of methyl alcohol and methyl acetate, and a small percentage of a wax.

10. A high speed paint and varnish remover possessing high initial surface wrinkling power capable of rapidly opening the surface to ingress of solvent, said remover containing furfural, a benzolic solvent selected from the group consisting of benzol and chlorbenzol, methyl acetate, and a small percentage of a wax.

15 20 BORIS N. LOUGOVY.

25

30

35

40

45

50

55

60

65